

Dec. 16, 1958

A. E. STRINGFELLOW

2,864,919

CERAMIC ARCING PLATE MATERIAL

Filed May 11, 1955

FIG. 1.



FIG. 2.

INVENTOR,  
ALLEN E. STRINGFELLOW

BY

Attdeauk & Faber  
ATTORNEYS

2,864,919

## CERAMIC ARCING PLATE MATERIAL

Allen E. Stringfellow, Haddonfield, N. J., assignor to  
I-T-E Circuit Breaker Company, Philadelphia, Pa., a  
corporation of Pennsylvania

Application May 11, 1955, Serial No. 507,632

2 Claims. (Cl. 200—144)

My invention relates to a novel ceramic composition to be used as the arc extinguishing means in connection with circuit interrupting equipment, and to arcing plates and an arc chute embodying this novel composition.

Circuit interrupting equipment, as is well known in the art must have arc extinguishing means in order to cool off and deionize the arc which is formed between the movable interrupting contacts.

For relatively low voltage application, the arc extinguishing means comprises a plurality of metallic members which, through their high heat conductivity, are used to cool the arc and to prevent restriking thereof. However, for high voltage circuit interrupting equipment, for which my invention is directed, it is necessary to use insulating plates which are interleaved so as to provide a tortuous path for the arc and thereby more rapidly extinguish the same.

A typical arrangement for such plates is disclosed in copending applications (C-233) Serial No. 322,027, now U. S. Patent No. 2,759,093, and (C-248) Serial No. 353,281 which are owned by applicant's assignee. Another arrangement which may be used is exemplified in my copending application (C-293) Serial No. 439,118. The ceramic insulating plates which have been used in such arc extinguishers in the past have comprised such materials as Transite, cold-molded asbestos, glass bonded mica and zircon.

The requirements for insulating plates of this type are such that they must be of a high dielectric strength having high resistance to thermal shock and must maintain their strength before and after interruption and not be subject to deterioration and erosion from repeated contact with high voltage arcs.

Some of the faults of the above mentioned materials are evident from the tabulation below.

| Material             | Strength Before Interruption | Strength After Interruption | Interrupting Ability | Deterioration, Erosion, etc. |
|----------------------|------------------------------|-----------------------------|----------------------|------------------------------|
| Transite             | Fair                         | Poor                        | Poor                 | Extreme.                     |
| Cold Molded Asbestos | do                           | do                          | do                   | Do.                          |
| Glass Bonded Mica    | Very Good                    | 43% Loss                    | Fair                 | Very High.                   |
| Zircon               | Good                         | 30-70% Loss                 | Very Good            | Very High.<br>{Too Extreme.  |

I propose to overcome these faults as well as other disadvantages in the ceramic arcing materials known to the prior art by providing an arcing plate made of a novel ceramic composition which will have outstanding interrupting ability, low strength loss during interruption and will incur very little deterioration through repeated contact with high voltage arcs. I have found that a plate meeting these requirements may be made from a composition containing a substantial quantity of cordierite crystals, specifically more than 50 percent of such crystals, having a specific ultimate composition which can be defined on the  $MgO-SiO_2-Al_2O_3$  phase diagram as 5 to 15 percent  $MgO$ , 22 to 58 percent  $Al_2O_3$  and 38 to 63

percent  $SiO_2$ . Preferably a more limited composition range may be included, which will contain a minimum of fifty percent cordierite crystals and have an ultimate analysis consisting essentially of 5 to 13 percent of  $MgO$ , 37 to 57 percent  $Al_2O_3$  and 38 to 50 percent of  $SiO_2$ .

Accordingly it is an object of my invention to provide as a novel ceramic arcing material a composition containing a substantial quantity of cordierite crystals and having an ultimate composition consisting essentially of specific proportions of  $MgO$ ,  $Al_2O_3$  and  $SiO_2$ .

It is another object of my invention to provide a novel ceramic arcing plate which will have outstanding interrupting ability, little loss in strength after interruption and be subject to very little deterioration and erosion from repeated use.

It is still another object of my invention to provide a novel method for preparing a cordierite-containing ceramic composition which will be suitable for use as a ceramic arcing plate or assembly of such plates in circuit interrupting equipment.

These and other objects of my invention will become more apparent when taken in connection with the description and the drawings in which:

Figure 1 shows the three (3) component diagram  $MgO-Al_2O_3-SiO_2$  and having a portion thereof outlined to show the specific ceramic composition which I have found particularly suitable in my ceramic arcing plates, and another small portion thereof outlined to point out a particularly preferred embodiment of my invention. The diagram is based on weight percentages of the three components and also indicates the point at which cordierite,  $2MgO \cdot 2Al_2O_3 \cdot 5SiO_2$  as well as other compounds containing these components will occur. By dotted lines, compatibility triangles are also outlined.

Figure 2 illustrates a typical ceramic arcing plate which may be made from my novel composition so that they would form what is known as an arc "chute." The plates as they appear in Figure 2 may be held in spaced-apart relationship by independent spacer means as shown in copending application (C-248) Serial No. 353,281 or may be integral as shown in my copending application (C-293) Serial No. 439,118.

Moreover, the plates may be flat or flanged as indicated in these respective copending applications.

Referring now to Figure 1, the novel composition which I propose to use in the ceramic arcing plates is bounded by the percentages, 5 to 15 percent  $MgO$ , 22 to 58 percent  $Al_2O_3$  to 38 and 63 percent  $SiO_2$ . This entire region is noted as area "A" and bounded by solid lines.

It includes the area "B" hereinafter referred to. These compositions have been found to provide arcing plates having very high heat shock resistance, low strength loss under interrupting conditions (0 to 10 percent after fifty short circuits) and very good interrupting ability.

The composition which I particularly prefer and which gives the best quality from all points considering interrupting ability, strength and ease of manufacture is bounded by the following coordinates of the phase diagram:

5 to 13 percent  $MgO$   
37 to 57 percent  $Al_2O_3$   
38 to 50 percent  $SiO_2$

This area is indicated in Figure 1 as area "B" and is outlined by the cross-hatched lines. This area is characterized by compositions having very low shrinkage values (between 0.6 and 2 percent), which makes the element easy to manufacture and relatively free from firing warpage, camber and cracks. These compositions give very high heat shock values and have high strength in the range of 10,000 to 11,000 p. s. i., which after 50 interruptions does not lower more than 2 to 5 percent of their initial strength. After this number of interruptions, arcing plates of this composition, although possibly having a lower initial strength than glass bonded mica are found to have strengths equal or better than this or other high strength materials of the prior art.

In the weight percent triaxial diagram of Figure 1, the various phases which may occur are shown and compatibility triangles connecting the indicated phases are outlined by the dotted lines.

Cordierite bodies are represented by a predominance of the compound  $2\text{MgO} \cdot 2\text{Al}_2\text{O}_3 \cdot 5\text{SiO}_2$  which is the composition of the cordierite crystal. They have an orthorhombic crystalline structure and are particularly important in my composition because of their very low coefficients of thermal expansion and their ability to withstand thermal shock. These cordierite crystals which appear in substantial amounts in my composition and preferably in amounts over 50 percent have been found to have a coefficient of thermal expansion of  $3 \times 10^{-6}$  or less for the range of 60 to 1110° F. The formation of the cordierite in a ceramic body in the ternary system  $\text{MgO} - \text{Al}_2\text{O}_3 - \text{SiO}_2$  occurs to a greater or lesser extent over a rather wide compositional area and varies radically with the firing temperature.

In order to produce the cordierite crystals, the range of temperatures which I prefer to use varies from about 2300 to 2700° F. dependent upon the composition of the body and the raw materials used. Increases in firing temperatures causes an increase in individual crystal size. However, temperatures which are too high cause the cordierite to dissociate into mullite and a low viscosity melt.

The following specific Examples A, B and C cover the most desirable range of properties of starting materials which are used in the formation of my ceramic composition:

|                           | A       | B       | C       |
|---------------------------|---------|---------|---------|
|                           | Percent | Percent | Percent |
| Sierramic Talc.....       | 35.0    | 34.4    | 25.0    |
| Edgar Plastic Kaolin..... | 36.1    | 46.8    | 53.0    |
| A-10 Alumina.....         | 28.9    | 18.8    | 22.0    |

These materials are further described as follows:

I. Sierramic Talc is a product of the Sierra Talc and Clay Company and commonly has the following analysis:

|                               | Percent |
|-------------------------------|---------|
| $\text{SiO}_2$ .....          | 59.62   |
| $\text{MgO}$ .....            | 29.91   |
| $\text{Al}_2\text{O}_3$ ..... | 2.05    |
| $\text{CaO}$ .....            | 0.01    |
| $\text{Fe}_2\text{O}_3$ ..... | 9.94    |
| $\text{K}_2\text{O}$ .....    | 0.49    |
| $\text{Na}_2\text{O}$ .....   | 5.48    |
| Loss on ignition.....         |         |

II. Edgar Plastic Kaolin is a product of the Edgar Florida, Hammil & Gillespie, Inc., New York, and commonly has the following analysis:

|                               | Percent |
|-------------------------------|---------|
| $\text{SiO}_2$ .....          | 46.95   |
| $\text{Al}_2\text{O}_3$ ..... | 36.75   |
| $\text{MgO}$ .....            | 0.20    |
| $\text{CaO}$ .....            | 0.80    |
| $\text{K}_2\text{O}$ .....    | 0.24    |
| $\text{Na}_2\text{O}$ .....   | 0.18    |
| $\text{TiO}_2$ .....          |         |
| Loss on ignition.....         | 14.95   |

III. A-10 Alumina is a product of the Aluminum

Company of America and commonly has the following analysis:

|                               | Percent |
|-------------------------------|---------|
| $\text{Al}_2\text{O}_3$ ..... | 99.68   |
| $\text{SiO}_2$ .....          | 0.04    |
| Misc.....                     | 0.28    |

|    | Oxide Composition             | Percent |      |
|----|-------------------------------|---------|------|
| 10 | $\text{MgO}$ .....            | 11.5    | 8.5  |
|    | $\text{Al}_2\text{O}_3$ ..... | 47.0    | 44.0 |
|    | $\text{SiO}_2$ .....          | 41.5    | 47.5 |

From the examples above it can be seen that I particularly prefer that the starting composition falling within the cross-hatched area of Figure 1 should contain the following:

|                           | Percent |
|---------------------------|---------|
| Sierramic Talc.....       | 25-35   |
| Edgar Plastic Kaolin..... | 36-53   |
| A-10 Alumina.....         | 22-29   |

Oxide composition:

|    |                               |           |
|----|-------------------------------|-----------|
| 25 | $\text{MgO}$ .....            | 8.5-11.5  |
|    | $\text{Al}_2\text{O}_3$ ..... | 41-47     |
|    | $\text{SiO}_2$ .....          | 41.5-47.5 |

To illustrate a specific embodiment of the method for forming the cordierite crystals the following procedure is employed:

The raw clays are blended in a Simpson Mix-Muller with 4 percent water and 4 percent binder. The binder may be any of the commonly known organic binders which have long been used in the firing of ceramic objects. Binders of this type are temporary in that they are either partially or completely burned out of the body upon firing. An example of a suitable binder would be a hemicellulose extract such as that going under the trade name "Masonoid." Another example would be methyl cellulose (see Pat. No. 2,358,407). This blend is screened through a 50 mesh screen to give additional mixing and break up any lumps. The blend is then compressed at 10,000 p. s. i. and then fired at 2534° F.

Figure 2 illustrates a ceramic arcing plate made of my novel composition and illustrates how the individual plates may be interleaved. The ceramic plate illustrated therein contains a notch cut vertically through the plate and arranged on one side of the vertical center line of the plate. Thus, the plate is divided into a wider segment 11 and a narrower segment 12. These plates are resiliently mounted in the circuit interrupter and are interleaved so that the segments would appear alternately when viewing either the right or left hand side of the stack. Thus an arc must follow an elongated meandering path in order to pass through a stack of interleaved plates. These dielectric plates, so arranged, provide what is known as an arc "chute." The dotted lines in Figure 1 are indicative of changes in phase. In other words any point lying within an area defined by the dotted lines will contain a composition having phase mixtures of the compounds noted by the apices of the triangles defined by these dotted lines.

As previously mentioned and pointed out in the co-pending applications hereinbefore referred to, these arcing plates may be flat as shown or strengthened, spaced and supported by providing them with ribs or flanges adjacent to each of the elongated sides of the plates and extending along substantially the full length of each side, in the manner set forth in my copending application Serial No. 439,118. The flanges may be one or both surfaces of the plate depending on whether an I-shaped or U-shaped cross-section is desired.

70 Although Figure 2 illustrates the staggered interleaved relationship of the plates it is clear that it is within the scope and the spirit of my invention to include an assembly which contains any feasible number of plates so shown. The arrangement of plates, however, should provide the necessary tortuous path for the arc.

Arc chutes containing a plate assembly in which the plates have been composed of my novel ceramic composition have been shown, through various tests, to be superior to plates made of materials used in the prior art. For example, interruption tests on high voltage breakers have proven that plates of my novel composition have increased the interrupting rating over 90 percent over glass bonded mica and even more over the Transite type plates.

Moreover, the cordierite arcing material of the type herein disclosed and claimed have been found to give much better results under spalling tests. Apparently, my cordierite plates cool and heat more evenly so that less of a temperature gradient is set up during the arc extinguishing process thereby preventing variations in the coefficient of thermal expansion between the surface layer and the inner portion of the body which have often been found great enough to shear off the surface layer and thus result in spalling.

I do not intend to limit the scope of my invention to the specific type of arcing plates herein disclosed. It should be clear to those skilled in the art that my novel ceramic composition is suitable for use in various types of electrical insulators which come in contact with high voltage arcs. These would include arc plates, tube for load switches, rods for load switches, tubes for air blast switches, arc chute liner plates, arc chute cooling plates and arc plate spacers.

In the foregoing, I have described my invention only in connection with preferred embodiments thereof. Many variations and modifications of the principles of my invention within the scope of the description herein are obvious. Accordingly, I prefer to be bound not by the specific disclosure herein, but only by the appending claims.

## I claim:

1. In a circuit interrupter arc chute, a plurality of ceramic arcing plates having a low coefficient of thermal expansion and high heat shock resistance after repeated circuit interruptions, means for supporting and maintaining said plates in an interleaved, spaced-apart relationship so that an arc must follow an elongated path to pass through a stack of said plates, said plates being composed of a ceramic material consisting essentially of 5 to 13 percent MgO, 37 to 57 percent Al<sub>2</sub>O<sub>3</sub> and 38 to 50 percent SiO<sub>2</sub> and containing more than 50 percent cordierite crystals.

2. In a circuit interrupter arc chute, a plurality of ceramic arcing plates having a low coefficient of thermal expansion and high heat shock resistance after repeated circuit interruptions, means for supporting and maintaining said plates in an interleaved, spaced-apart relationship so that an arc must follow an elongated path to pass through a stack of said plates, said plates being composed of a ceramic material consisting essentially of 8.5 to 11.5 percent MgO, 41 to 47 percent Al<sub>2</sub>O<sub>3</sub> and 41.5 to 47.5 percent SiO<sub>2</sub> and containing more than 50 percent cordierite crystals.

## References Cited in the file of this patent

## UNITED STATES PATENTS

2,036,190 Benner et al. ----- Apr. 7, 1936

## FOREIGN PATENTS

109,919 Australia ----- 1940

## OTHER REFERENCES

Journal of the American Ceramic Society, vol. 30, 35 1947, part II, page 79.